



US009469939B2

(12) **United States Patent**  
**Ardiff et al.**

(10) **Patent No.:** **US 9,469,939 B2**  
(45) **Date of Patent:** **\*Oct. 18, 2016**

(54) **METHOD TO CREATE AN ENVIRONMENTALLY RESISTANT SOFT ARMOR COMPOSITE**

(75) Inventors: **Henry G. Ardiff**, Chesterfield, VA (US); **Ralf Klein**, Midlothian, VA (US); **Brian D. Arvidson**, Chester, VA (US); **Ashok Bhatnagar**, Richmond, VA (US); **Lori L. Wagner**, Richmond, VA (US)

(73) Assignee: **HONEYWELL INTERNATIONAL INC.**, Morris Plains, NJ (US)

(\*) Notice: Subject to any disclaimer, the term of this patent is extended or adjusted under 35 U.S.C. 154(b) by 471 days.

This patent is subject to a terminal disclaimer.

(21) Appl. No.: **12/970,493**

(22) Filed: **Dec. 16, 2010**

(65) **Prior Publication Data**

US 2012/0156952 A1 Jun. 21, 2012

**Related U.S. Application Data**

(63) Continuation-in-part of application No. 11/729,258, filed on Mar. 28, 2007, now Pat. No. 7,875,563.

(51) **Int. Cl.**

**B32B 27/04** (2006.01)  
**D06N 3/18** (2006.01)

(Continued)

(52) **U.S. Cl.**

CPC ..... **D06N 3/183** (2013.01); **D21H 19/80** (2013.01); **D21H 27/001** (2013.01); **D21H 27/30** (2013.01); **F41H 5/0478** (2013.01); **D06N 2209/103** (2013.01); **D06N 2213/03** (2013.01); **Y10T 442/2623** (2015.04)

(58) **Field of Classification Search**

CPC ..... D06N 3/18; D06N 3/183; D06N 2213/00  
USPC ..... 442/64, 59, 60, 82, 83, 88, 89, 92, 94, 442/134, 135; 428/114; 89/36.01, 36.05  
See application file for complete search history.

(56) **References Cited**

U.S. PATENT DOCUMENTS

4,467,005 A 8/1984 Pusch et al. .... 428/111  
4,529,633 A 7/1985 Karlsson ..... 428/17  
(Continued)

FOREIGN PATENT DOCUMENTS

EP 169432 A1 \* 1/1986  
GB 1369285 10/1974

(Continued)

OTHER PUBLICATIONS

Kevlar Aramid Fiber Technical Guide, DuPont, p. II-1.\*  
(Continued)

*Primary Examiner* — Jennifer Chriss

*Assistant Examiner* — Frank Vineis

(74) *Attorney, Agent, or Firm* — Roberts & Roberts, LLP; Richard S. Roberts, Jr.

(57) **ABSTRACT**

Fibrous substrates and articles that retain their superior ballistic resistance performance after exposure to liquids such as sea water and organic solvents, such as gasoline and other petroleum-based products. The fibrous substrates are coated with a multilayer polymeric coating including at least two polymer layers wherein the first polymer and the second polymer forming said respective layers are the same and optionally comprise fluorine.

**10 Claims, 1 Drawing Sheet**



|      |                   |           |  |  |                  |         |                            |
|------|-------------------|-----------|--|--|------------------|---------|----------------------------|
| (51) | <b>Int. Cl.</b>   |           |  |  |                  |         |                            |
|      | <i>F41H 5/04</i>  | (2006.01) |  |  | 2008/0237911 A1  | 10/2008 | Ardiff et al. .... 264/129 |
|      | <i>D21H 19/80</i> | (2006.01) |  |  | 2008/0241494 A1  | 10/2008 | Ardiff et al. .... 428/219 |
|      | <i>D21H 27/00</i> | (2006.01) |  |  | 2009/0163098 A1* | 6/2009  | Ardiff et al. .... 442/164 |
|      | <i>D21H 27/30</i> | (2006.01) |  |  | 2009/0163105 A1* | 6/2009  | Ardiff et al. .... 442/399 |

(56) **References Cited**

## U.S. PATENT DOCUMENTS

|                  |         |                         |                      |
|------------------|---------|-------------------------|----------------------|
| 4,623,574 A *    | 11/1986 | Harpell et al. ....     | 428/113              |
| 4,680,221 A      | 7/1987  | Murayama et al. ....    | 442/126              |
| 4,913,978 A      | 4/1990  | Klotz et al. ....       | 428/551              |
| 5,229,199 A      | 7/1993  | Miner et al. ....       | 442/135              |
| 5,357,726 A      | 10/1994 | Effenberger et al. .... | 52/309.7             |
| 5,409,557 A *    | 4/1995  | Mammino et al. ....     | 156/137              |
| 5,587,230 A      | 12/1996 | Lin et al. ....         | 442/135              |
| 6,034,004 A *    | 3/2000  | Fels ....               | F41H 1/02<br>428/911 |
| 6,326,094 B1     | 12/2001 | Asano et al. ....       | 428/38               |
| 6,335,094 B1     | 1/2002  | Owaki et al. ....       | 428/374              |
| 6,642,159 B1     | 11/2003 | Bhatnagar et al. ....   | 442/134              |
| 6,838,401 B1     | 1/2005  | Murayama et al. ....    | 442/335              |
| 7,407,899 B2     | 8/2008  | Wang et al. ....        | 442/93               |
| 2004/0018787 A1  | 1/2004  | Bullock et al. ....     | 442/59               |
| 2005/0272334 A1* | 12/2005 | Wang et al. ....        | 442/93               |
| 2005/0282007 A1* | 12/2005 | Sauer ....              | B32B 5/26<br>428/357 |

## FOREIGN PATENT DOCUMENTS

|    |                    |         |
|----|--------------------|---------|
| JP | 2002-316319        | 10/2002 |
| JP | 2005126885         | 5/2005  |
| WO | WO 0196695         | 12/2001 |
| WO | WO 0214408         | 2/2002  |
| WO | WO 2004023060 A1 * | 3/2004  |
| WO | WO 2006/132852     | 12/2006 |

## OTHER PUBLICATIONS

Dupont, Kevlar, archived Feb. 5, 2006, [http://www2.dupont.com/Products/en\\_RU/Kevlar\\_en.html](http://www2.dupont.com/Products/en_RU/Kevlar_en.html).\*

Mahfuz, H., Enhanced stab resistance of armor composites with functionalized silica nanoparticles, Journal of Applied Physics 105, 064307, Mar. 18, 2009.\*

Yang, Comprehensive Composite Materials, vol. 1; 2000; pp. 199-229.\*

\* cited by examiner



**METHOD TO CREATE AN  
ENVIRONMENTALLY RESISTANT SOFT  
ARMOR COMPOSITE**

**CROSS-REFERENCE TO RELATED  
APPLICATION**

This application is a Continuation-In-Part of U.S. patent application Ser. No. 11/729,258 filed Mar. 28, 2007, now U.S. Pat. No. 7,875,563, the entire disclosure of which is incorporated by reference herein.

**BACKGROUND OF THE INVENTION**

**1. Field of the Invention**

This invention relates to ballistic resistant articles having excellent resistance to deterioration due to liquid exposure. More particularly, the invention pertains to ballistic resistant fabrics and articles that retain their superior ballistic resistance performance after exposure to liquids such as sea water and organic solvents, such as gasoline and other petroleum-based products.

**2. Description of the Related Art**

Ballistic resistant articles containing high strength fibers that have excellent properties against projectiles are well known. Articles such as bullet resistant vests, helmets, vehicle panels and structural members of military equipment are typically made from fabrics comprising high strength fibers. High strength fibers conventionally used include polyethylene fibers, aramid fibers such as poly(phenylene-diamine terephthalamide), graphite fibers, nylon fibers, glass fibers and the like. For many applications, such as vests or parts of vests, the fibers may be used in a woven or knitted fabric. For other applications, the fibers may be encapsulated or embedded in a polymeric matrix material to form woven or non-woven rigid or flexible fabrics.

Various ballistic resistant constructions are known that are useful for the formation of hard or soft armor articles such as helmets, panels and vests. For example, U.S. Pat. Nos. 4,403,012, 4,457,985, 4,613,535, 4,623,574, 4,650,710, 4,737,402, 4,748,064, 5,552,208, 5,587,230, 6,642,159, 6,841,492, 6,846,758, all of which are incorporated herein by reference, describe ballistic resistant composites which include high strength fibers made from materials such as extended chain ultra-high molecular weight polyethylene. These composites display varying degrees of resistance to penetration by high speed impact from projectiles such as bullets, shells, shrapnel and the like.

For example, U.S. Pat. Nos. 4,623,574 and 4,748,064 disclose simple composite structures comprising high strength fibers embedded in an elastomeric matrix. U.S. Pat. No. 4,650,710 discloses a flexible article of manufacture comprising a plurality of flexible layers comprised of high strength, extended chain polyolefin (ECP) fibers. The fibers of the network are coated with a low modulus elastomeric material. U.S. Pat. Nos. 5,552,208 and 5,587,230 disclose an article and method for making an article comprising at least one network of high strength fibers and a matrix composition that includes a vinyl ester and diallyl phthalate. U.S. Pat. No. 6,642,159 discloses an impact resistant rigid composite having a plurality of fibrous layers which comprise a network of filaments disposed in a matrix, with elastomeric layers there between. The composite is bonded to a hard plate to increase protection against armor piercing projectiles.

Hard or rigid body armor provides good ballistic resistance, but can be very stiff and bulky. Accordingly, body

armor garments, such as ballistic resistant vests, are preferably formed from flexible or soft armor materials. However, while such flexible or soft materials exhibit excellent ballistic resistance properties, they also generally exhibit poor resistance to liquids, including fresh water, seawater and organic solvents, such as petroleum, gasoline, gun lube and other solvents derived from petroleum. This is problematic because the ballistic resistance performance of such materials is generally known to deteriorate when exposed to or submerged in liquids. Further, while it has been known to apply a protective film to a fabric surface to enhance fabric durability and abrasion resistance, as well as water or chemical resistance, these films add weight to the fabric. Accordingly, it would be desirable in the art to provide soft, flexible ballistic resistant materials that perform at acceptable ballistic resistance standards after being contacted with or submerged in a variety of liquids, and also have superior durability without the use of a protective surface film in addition to a binder polymer coating.

Few conventional binder materials, commonly referred to in the art as polymeric "matrix" materials, are capable of providing all the desired properties discussed herein, particularly when applied as a single layer or coating. Said properties are improved when applied as multiple layers and/or multiple coatings.

In addition, fluorine-containing polymers are known to be desirable in other arts due to their resistance to dissolution, penetration and/or transpiration by sea water and resistance to dissolution, penetration and/or transpiration by one or more organic solvents, such as diesel gasoline, non-diesel gasoline, gun lube, petroleum and organic solvents derived from petroleum. In the art of ballistic resistant materials, it has been discovered that fluorine-containing coatings advantageously contribute to the retention of the ballistic resistance properties of a ballistic resistant fabric after prolonged exposure to potentially harmful liquids, eliminating the need for a protective surface film to achieve such benefits. Beneficially, fluorine-containing polymers offers the desired protection from liquids, as well as heat and cold resistance, and resistance to abrasion and wear, while maintaining good flexibility and superior ballistic resistance properties.

The present invention provides a ballistic resistant fabric which is formed with multiple layers of a polymeric binder material wherein a first polymer layer comprises a first polymer and a second polymer layer on said first polymer layer comprises a second polymer, wherein the first polymer and the second polymer are the same and both optionally comprise fluorine. The polymer layers are preferably contacted with each other as liquids to facilitate their miscibility and adhesion at their contact interfaces.

**SUMMARY OF THE INVENTION**

The invention provides a ballistic resistant fibrous composite comprising at least one fibrous substrate having a multilayer coating thereon, wherein said fibrous substrate comprises one or more fibers having a tenacity of about 7 g/denier or more and a tensile modulus of about 150 g/denier or more; said multilayer coating comprising a first polymer layer on a surface of said one or more fibers, said first polymer layer comprising a first polymer, and a second polymer layer on said first polymer layer, said second polymer layer comprising a second polymer, wherein the first polymer and the second polymer are the same and optionally comprise fluorine.

The invention also provides a method of forming a ballistic resistant fibrous composite comprising:

- a) providing at least one fibrous substrate having a surface; wherein said at least one fibrous substrate comprises one or more fibers having a tenacity of about 7 g/denier or more and a tensile modulus of about 150 g/denier or more;
  - b) applying a first polymer layer onto the surface of the at least one fibrous substrate, said first polymer layer comprising a first polymer;
  - c) thereafter, applying a second polymer layer onto the first polymer layer, said second polymer layer comprising a second polymer;
- and wherein the first polymer and the second polymer are the same and optionally comprise fluorine.

Also provided are articles formed from the fibrous composites of the invention.

#### BRIEF DESCRIPTION OF THE DRAWING

FIG. 1 is a schematic representation illustrating a process for applying a multilayer coating onto a fibrous substrate utilizing a hybrid coating technique.

#### DETAILED DESCRIPTION OF THE INVENTION

The invention presents fibrous composites and articles that retain superior ballistic penetration resistance after exposure to water, particularly sea water, and organic solvents, particularly solvents derived from petroleum such as gasoline. Particularly, the invention provides fibrous composites formed by applying a multilayer coating onto at least one fibrous substrate. A fibrous substrate is considered to be a single fiber in most embodiments, but may alternately be considered a fabric when a plurality of fibers are united as a monolithic structure prior to application of the multilayer coating, such as with a woven fabric that comprises a plurality of woven fibers. The method of the invention may also be conducted on a plurality of fibers that are arranged as a fiber web or other arrangement, which are not technically considered to be a fabric at the time of coating, and is described herein as coating on a plurality of fibrous substrates. The invention also provides fabrics formed from a plurality of coated fibers and articles formed from said fabrics.

The fibrous substrates of the invention are coated with a multilayer coating that comprises at least two polymer layers. Specifically, the multilayer coatings comprise a first polymer layer on a surface of the fibers, said first polymer layer comprising a first polymer, and a second polymer layer on the first polymer layer, said second polymer layer comprising a second polymer, wherein the first polymer and the second polymer are the same and optionally comprise fluorine, i.e. optionally comprise at least one fluorine-containing polymer. As used herein, a “fluorine-containing” polymer or fluorine-containing polymeric binder describes a material formed from at least one polymer that includes fluorine atoms. Such include fluoropolymers and/or fluorocarbon-containing materials, i.e. fluorocarbon resins. A “fluorocarbon resin” generally refers to polymers including fluorocarbon groups.

For the purposes of the invention, articles that have superior ballistic penetration resistance describe those which exhibit excellent properties against high speed projectiles. The articles also exhibit excellent resistance properties against fragment penetration, such as shrapnel. For the purposes of the present invention, a “fiber” is an elongate body the length dimension of which is much greater than the transverse dimensions of width and thickness. The cross-

sections of fibers for use in this invention may vary widely. They may be circular, flat or oblong in cross-section. Accordingly, the term fiber includes filaments, ribbons, strips and the like having regular or irregular cross-section.

5 They may also be of irregular or regular multi-lobial cross-section having one or more regular or irregular lobes projecting from the linear or longitudinal axis of the fibers. It is preferred that the fibers are single lobed and have a substantially circular cross-section.

10 As stated above, the multilayer coatings may be applied onto a single polymeric fiber or a plurality of polymeric fibers. A plurality of fibers may be present in the form of a fiber web, a woven fabric, a non-woven fabric or a yarn, where a yarn is defined herein as a strand consisting of multiple fibers and where a fabric comprises a plurality of united fibers. In embodiments including a plurality of fibers, the multilayer coatings may be applied either before the fibers are arranged into a fabric or yarn, or after the fibers are arranged into a fabric or yarn.

15 20 The fibers of the invention may comprise any polymeric fiber type. Most preferably, the fibers comprise high strength, high tensile modulus fibers which are useful for the formation of ballistic resistant materials and articles. As used herein, a “high-strength, high tensile modulus fiber” is one which has a preferred tenacity of at least about 7 g/denier or more, a preferred tensile modulus of at least about 150 g/denier or more, and preferably an energy-to-break of at least about 8 J/g or more, each both as measured by ASTM D2256. As used herein, the term “denier” refers to the unit of linear density, equal to the mass in grams per 9000 meters of fiber or yarn. As used herein, the term “tenacity” refers to the tensile stress expressed as force (grams) per unit linear density (denier) of an unstressed specimen. The “initial modulus” of a fiber is the property of 25 30 35 a material representative of its resistance to deformation. The term “tensile modulus” refers to the ratio of the change in tenacity, expressed in grams-force per denier (g/d) to the change in strain, expressed as a fraction of the original fiber length (in/in). The polymers forming the fibers are preferably high-strength, high tensile modulus fibers suitable for the manufacture of ballistic resistant fabrics. Particularly suitable high-strength, high tensile modulus fiber materials that is particularly suitable for the formation of ballistic

40 45 50 55 60 resistant materials and articles include polyolefin fibers including high density and low density polyethylene. Particularly preferred are extended chain polyolefin fibers, such as highly oriented, high molecular weight polyethylene fibers, particularly ultra-high molecular weight polyethylene fibers, and polypropylene fibers, particularly ultra-high molecular weight polypropylene fibers. Also suitable are aramid fibers, particularly para-aramid fibers, polyamide fibers, polyethylene terephthalate fibers, polyethylene naphthalate fibers, extended chain polyvinyl alcohol fibers, extended chain polyacrylonitrile fibers, polybenzazole fibers, such as polybenzoxazole (PBO) and polybenzothiazole (PBT) fibers, liquid crystal copolyester fibers and rigid rod fibers such as M5® fibers. Each of these fiber types is conventionally known in the art. Also suitable for producing polymeric fibers are copolymers, block polymers and blends of the above materials.

The most preferred fiber types for ballistic resistant fabrics include polyethylene, particularly extended chain polyethylene fibers, aramid fibers, polybenzazole fibers, liquid crystal copolyester fibers, polypropylene fibers, particularly 65 highly oriented extended chain polypropylene fibers, polyvinyl alcohol fibers, polyacrylonitrile fibers and rigid rod fibers, particularly M5® fibers.

In the case of polyethylene, preferred fibers are extended chain polyethylenes having molecular weights of at least 500,000, preferably at least one million and more preferably between two million and five million. Such extended chain polyethylene (ECPE) fibers may be grown in solution spinning processes such as described in U.S. Pat. No. 4,137,394 or 4,356,138, which are incorporated herein by reference, or may be spun from a solution to form a gel structure, such as described in U.S. Pat. Nos. 4,551,296 and 5,006,390, which are also incorporated herein by reference. A particularly preferred fiber type for use in the invention are polyethylene fibers sold under the trademark SPECTRA® from Honeywell International Inc. SPECTRA® fibers are well known in the art and are described, for example, in U.S. Pat. Nos. 4,623,547 and 4,748,064.

Also particularly preferred are aramid (aromatic polyamide) or para-aramid fibers. Such are commercially available and are described, for example, in U.S. Pat. No. 3,671,542. For example, useful poly(p-phenylene terephthalamide) filaments are produced commercially by Dupont Corporation under the trademark of KEVLAR®. Also useful in the practice of this invention are poly(m-phenylene isophthalamide) fibers produced commercially by Dupont under the trademark NOMEX® and fibers produced commercially by Teijin under the trademark TWARON®; aramid fibers produced commercially by Kolon Industries, Inc. of Korea under the trademark HERACRON®; p-aramid fibers SVM™ and RUSART™ which are produced commercially by Kamensk Volokno JSC of Russia and ARMOST™ p-aramid fibers produced commercially by JSC Chim Volokno of Russia.

Suitable polybenzazole fibers for the practice of this invention are commercially available and are disclosed for example in U.S. Pat. Nos. 5,286,833, 5,296,185, 5,356,584, 5,534,205 and 6,040,050, each of which is incorporated herein by reference. Preferred polybenzazole fibers are ZYLON® brand fibers from Toyobo Co. Suitable liquid crystal copolyester fibers for the practice of this invention are commercially available and are disclosed, for example, in U.S. Pat. Nos. 3,975,487; 4,118,372 and 4,161,470, each of which is incorporated herein by reference. Suitable polypropylene fibers include highly oriented extended chain polypropylene (ECPP) fibers as described in U.S. Pat. No. 4,413,110, which is incorporated herein by reference. Suitable polyvinyl alcohol (PV-OH) fibers are described, for example, in U.S. Pat. Nos. 4,440,711 and 4,599,267 which are incorporated herein by reference. Suitable polyacrylonitrile (PAN) fibers are disclosed, for example, in U.S. Pat. No. 4,535,027, which is incorporated herein by reference. Each of these fiber types is conventionally known and is widely commercially available.

The other suitable fiber types for use in the present invention include rigid rod fibers such as M5® fibers, and combinations of all the above materials, all of which are commercially available. For example, the fibrous layers may be formed from a combination of SPECTRA® fibers and Kevlar® fibers. M5® fibers are formed from pyridobisimidazole-2,6-diyl (2,5-dihydroxy-p-phenylene) and are manufactured by Magellan Systems International of Richmond, Va. and are described, for example, in U.S. Pat. Nos. 5,674,969, 5,939,553, 5,945,537, and 6,040,478, each of which is incorporated herein by reference. Specifically preferred fibers include M5® fibers, polyethylene SPECTRA® fibers, aramid Kevlar® fibers and aramid TWARON® fibers. The fibers may be of any suitable denier, such as, for example, 50 to about 3000 denier, more preferably from about 200 to 3000 denier, still more preferably from about

650 to about 2000 denier, and most preferably from about 800 to about 1500 denier. The selection is governed by considerations of ballistic effectiveness and cost. Finer fibers are more costly to manufacture and to weave, but can produce greater ballistic effectiveness per unit weight.

The most preferred fibers for the purposes of the invention are either high-strength, high tensile modulus extended chain polyethylene fibers or high-strength, high tensile modulus para-aramid fibers. As stated above, a high-strength, high tensile modulus fiber is one which has a preferred tenacity of about 7 g/denier or more, a preferred tensile modulus of about 150 g/denier or more and a preferred energy-to-break of about 8 J/g or more, each as measured by ASTM D2256. In the preferred embodiment of the invention, the tenacity of the fibers should be about 15 g/denier or more, preferably about 20 g/denier or more, more preferably about 25 g/denier or more and most preferably about 30 g/denier or more. The fibers of the invention also have a preferred tensile modulus of about 300 g/denier or more, more preferably about 400 g/denier or more, more preferably about 500 g/denier or more, more preferably about 1,000 g/denier or more and most preferably about 1,500 g/denier or more. The fibers of the invention also have a preferred energy-to-break of about 15 J/g or more, more preferably about 25 J/g or more, more preferably about 30 J/g or more and most preferably have an energy-to-break of about 40 J/g or more.

These combined high strength properties are obtainable by employing well known processes. U.S. Pat. Nos. 4,413,110, 4,440,711, 4,535,027, 4,457,985, 4,623,547 4,650,710 and 4,748,064 generally discuss the formation of preferred high strength, extended chain polyethylene fibers employed in the present invention. Such methods, including solution grown or gel fiber processes, are well known in the art. Methods of forming each of the other preferred fiber types, including para-aramid fibers, are also conventionally known in the art, and the fibers are commercially available.

In accordance with the invention, a multilayer coating is applied onto at least part of a surface of the fiber or fabric substrates described herein. The multilayer coating comprises a first polymer layer directly on a surface of said fibers, and a second polymer layer on said first polymer layer, wherein the first polymer and the second polymer comprise or consist essentially of or consist of the same polymer. Each of the first polymer layer and the second polymer layer may have differences such as the presence or absence of a filler or other additive material, or may differ from each other in size or thickness, but in accordance with the invention the first polymer layer is formed from a first polymer that comprises a single polymer, a single copolymer or a polymer mixture that is substantially the same as the second polymer that forms the second polymer layer, wherein the second polymer thus also comprises a single polymer, a single co-polymer or a polymer mixture. The first polymer and/or second polymer may function as a binder material that binds a plurality of fibers together by way of their adhesive characteristics or after being subjected to well known heat and/or pressure conditions. In accordance with the invention, the first polymer forming said first polymer layer and the second polymer forming said second polymer layer, preferably comprise at least one fluorine-containing polymer. Additional polymer layers may also be coated onto the fibers, where each additional polymer layer is coated onto the last applied polymer layer. The optional additional polymer layers may be the same as or different than the first polymer layer and/or the second polymer layer.

It has been found that polymers containing fluorine atoms, particularly fluoropolymers and/or a fluorocarbon resins, are desirable because of their resistance to dissolution, permeation and/or transpiration by water and resistance to dissolution, permeation and/or transpiration by one or more organic solvents. Importantly, when fluorine-containing polymers are applied onto ballistic resistant fibers together with another polymeric material that is conventionally used in the art of ballistic resistant fabrics as a polymeric matrix material, the ballistic performance of a ballistic resistant composite formed therefrom is substantially retained after the composite is immersed in either water, e.g. salt water, or gasoline. Such materials also have a significantly reduced tendency to absorb either salt water or gasoline compared to fabrics formed without a fluorine-containing polymer layer, as the fluorine-containing polymer serves as a barrier between individual filaments, fibers and/or fabrics and salt water or gasoline.

Fluorine-containing materials, particularly fluoropolymers and fluorocarbon resin materials, are commonly known for their excellent chemical resistance and moisture barrier properties. Useful fluoropolymer and fluorocarbon resin materials herein include fluoropolymer homopolymers, fluoropolymer copolymers or blends thereof as are well known in the art and are described in, for example, U.S. Pat. Nos. 4,510,301, 4,544,721 and 5,139,878. Examples of useful fluoropolymers include, but are not limited to, homopolymers and copolymers of chlorotrifluoroethylene, ethylene-chlorotrifluoroethylene copolymers, ethylene-tetrafluoroethylene copolymers, fluorinated ethylene-propylene copolymers, perfluoroalkoxyethylene, polychlorotrifluoroethylene, polytetrafluoroethylene, polyvinyl fluoride, polyvinylidene fluoride, and copolymers and blends thereof.

As used herein, copolymers include polymers having two or more monomer components. Preferred fluoropolymers include homopolymers and copolymers of polychlorotrifluoroethylene. Particularly preferred are polychlorotrifluoroethylene (PCTFE) homopolymer materials sold under the ACLON™ trademark and which are commercially available from Honeywell International Inc. of Morristown, N.J. The most preferred fluoropolymers or fluorocarbon resins include fluorocarbon-modified polymers, particularly fluoro-oligomers and fluoropolymers formed by grafting fluorocarbon side-chains onto conventional polyethers (i.e. fluorocarbon-modified polyethers), polyesters (i.e. fluorocarbon-modified polyesters), polyanions (i.e. fluorocarbon-modified polyanions) such as polyacrylic acid (i.e. fluorocarbon-modified polyacrylic acid) or polyacrylates (i.e. fluorocarbon-modified polyacrylates), and polyurethanes (i.e. fluorocarbon-modified polyurethanes). These fluorocarbon side chains or perfluoro compounds are generally produced by a telomerization process and are referred to as C<sub>8</sub> fluorocarbons. For example, a fluoropolymer or fluorocarbon resin may be derived from the telomerization of an unsaturated fluoro-compound, forming a fluorotelomer, where said fluorotelomer is further modified to allow reaction with a polyether, polyester, polyanion, polyacrylic acid, polyacrylate or polyurethane, and where the fluorotelomer is then grafted onto a polyether, polyester, polyanion, polyacrylic acid, polyacrylate or polyurethane. Good representative examples of these fluorocarbon-containing polymers are NUVA® fluoropolymer products, commercially available from Clariant International, Ltd. of Switzerland. Other fluorocarbon resins, fluoro-oligomers and fluoropolymers having perfluoro acid-based and perfluoro alcohol-based side chains are also most preferred. Fluoropolymers and fluorocarbon resins having fluorocarbon side chains of

shorter lengths, such as C<sub>6</sub>, C<sub>4</sub> or C<sub>2</sub>, are also suitable, such as POLYFOX™ fluorochemicals, commercially available from Omnova Solutions, Inc. of Fairlawn, Ohio.

The fluorine-containing polymeric material may also 5 comprise a combination of a fluoropolymer or a fluorocarbon-containing material with another polymer, including blends of fluorine-containing polymeric materials with conventional polymeric binder (matrix) materials such as those described herein. In one preferred embodiment, the polymer 10 layer comprising a fluorine-containing polymer is a blend of a fluorine-containing polymer and an acrylic polymer. Preferred acrylic polymers non-exclusively include acrylic acid esters, particularly acrylic acid esters derived from monomers such as methyl acrylate, ethyl acrylate, n-propyl acrylate, 2-propyl acrylate, n-butyl acrylate, 2-butyl acrylate and tert-butyl acrylate, hexyl acrylate, octyl acrylate and 2-ethylhexyl acrylate. Preferred acrylic polymers also particularly include methacrylic acid esters derived from monomers such as methyl methacrylate, ethyl methacrylate, n-propyl methacrylate, 2-propyl methacrylate, n-butyl methacrylate, 2-butyl methacrylate, tert-butyl methacrylate, hexyl methacrylate, octyl methacrylate and 2-ethylhexyl methacrylate. Copolymers and terpolymers made from any of these constituent monomers are also preferred, along with those also 20 incorporating acrylamide, n-methylol acrylamide, acrylonitrile, methacrylonitrile, acrylic acid and maleic anhydride. Also suitable are modified acrylic polymers modified with non-acrylic monomers. For example, acrylic copolymers 25 and acrylic terpolymers incorporating suitable vinyl monomers such as: (a) olefins, including ethylene, propylene and isobutylene; (b) styrene, N-vinylpyrrolidone and vinylpyridine; (c) vinyl ethers, including vinyl methyl ether, vinyl ethyl ether and vinyl n-butyl ether; (d) vinyl esters of 30 aliphatic carboxylic acids, including vinyl acetate, vinyl propionate, vinyl butyrate, vinyl laurate and vinyl decanoates; and (f) vinyl halides, including vinyl chloride, vinylidene chloride, ethylene dichloride and propenyl chloride. Vinyl monomers which are likewise suitable are maleic 35 acid diesters and fumaric acid diesters, in particular of monohydric alkanols having 2 to 10 carbon atoms, preferably 3 to 8 carbon atoms, including dibutyl maleate, dihexyl maleate, diethyl maleate, dibutyl fumarate, dihexyl fumarate and diethyl fumarate.

40 Acrylic polymers and copolymers are preferred because of their inherent hydrolytic stability, which is due to the straight carbon backbone of these polymers. Acrylic polymers are also preferred because of the wide range of physical properties available in commercially produced materials. The range of physical properties available in acrylic resins 45 matches, and perhaps exceeds, the range of physical properties thought to be desirable in polymeric binder materials of ballistic resistant composite matrix resins.

The first polymer and second polymer layer may 50 alternately comprise a non-fluorine containing, i.e. substantially absent of fluorine, polymeric material that is conventionally employed in the art of ballistic resistant fabrics as a polymeric binder (matrix) material. A wide variety of conventional, non-fluorine-containing polymeric binder materials 55 are known in the art. Such include both low modulus, elastomeric materials and high modulus, rigid materials. Preferred low modulus, elastomeric materials are those having an initial tensile modulus less than about 6,000 psi (41.3 MPa), and preferred high modulus, rigid materials are those having an initial tensile modulus at least about 100,000 psi (689.5 MPa), each as measured at 37° C. by ASTM 60 D638. As used herein throughout, the term tensile modulus 65

means the modulus of elasticity as measured by ASTM 2256 for a fiber and by ASTM D638 for a polymeric binder material.

An elastomeric polymeric binder material may comprise a variety of materials. A preferred elastomeric binder material comprises a low modulus elastomeric material. For the purposes of this invention, a low modulus elastomeric material has a tensile modulus, measured at about 6,000 psi (41.4 MPa) or less according to ASTM D638 testing procedures. Preferably, the tensile modulus of the elastomer is about 4,000 psi (27.6 MPa) or less, more preferably about 2400 psi (16.5 MPa) or less, more preferably 1200 psi (8.23 MPa) or less, and most preferably is about 500 psi (3.45 MPa) or less. The glass transition temperature (T<sub>g</sub>) of the elastomer is preferably about 0° C. or less, more preferably about -40° C. or less, and most preferably about -50° C. or less. The elastomer also has a preferred elongation to break of at least about 50%, more preferably at least about 100% and most preferably has an elongation to break of at least about 300%.

A wide variety of materials and formulations having a low modulus may be utilized as a non-fluorine-containing polymeric binder material. Representative examples include polybutadiene, polyisoprene, natural rubber, ethylene-propylene copolymers, ethylene-propylene-diene terpolymers, polysulfide polymers, polyurethane elastomers, chlorosulfonated polyethylene, polychloroprene, plasticized polyvinylchloride, butadiene acrylonitrile elastomers, poly(isobutylene-co-isoprene), polyacrylates, polyesters, polyethers, silicone elastomers, copolymers of ethylene, and combinations thereof, and other low modulus polymers and copolymers. Also preferred are blends of different elastomeric materials, or blends of elastomeric materials with one or more thermoplastics.

Particularly useful are block copolymers of conjugated dienes and vinyl aromatic monomers. Butadiene and isoprene are preferred conjugated diene elastomers. Styrene, vinyl toluene and t-butyl styrene are preferred conjugated aromatic monomers. Block copolymers incorporating polyisoprene may be hydrogenated to produce thermoplastic elastomers having saturated hydrocarbon elastomer segments. The polymers may be simple tri-block copolymers of the type A-B-A, multi-block copolymers of the type (AB)<sub>n</sub> (n=2-10) or radial configuration copolymers of the type R-(BA)<sub>x</sub> (x=3-150); wherein A is a block from a polyvinyl aromatic monomer and B is a block from a conjugated diene elastomer. Many of these polymers are produced commercially by Kraton Polymers of Houston, Tex. and described in the bulletin "Kraton Thermoplastic Rubber", SC-68-81. The most preferred low modulus polymeric binder materials comprise styrenic block copolymers, particularly polystyrene-polyisoprene-polystyrene-block copolymers, sold under the trademark KRATON® commercially produced by Kraton Polymers and HYCAR® T122 acrylic resins commercially available from Noveon, Inc. of Cleveland, Ohio.

Preferred high modulus, rigid polymers include materials such as a vinyl ester polymer or a styrene-butadiene block copolymer, and also mixtures of polymers such as vinyl ester and diallyl phthalate or phenol formaldehyde and polyvinyl butyral. A particularly preferred high modulus material is a thermosetting polymer, preferably soluble in carbon-carbon saturated solvents such as methyl ethyl ketone, and possessing a high tensile modulus when cured of at least about  $1 \times 10^5$  psi (689.5 MPa) as measured by ASTM D638. Particularly preferred rigid materials are those described in U.S. Pat. No. 6,642,159, which is incorporated herein by reference.

Most preferred non-fluorine containing polymers comprise a polyurethane polymer, a polyether polymer, a polyester polymer, a polycarbonate resin, a polyacetal polymer, a polyamide polymer, a polybutylene polymer, an ethylene-vinyl acetate copolymer, an ethylene-vinyl alcohol copolymer, an ionomer, a styrene-isoprene copolymer, a styrene-butadiene copolymer, a styrene-ethylene/butylene copolymer, a styrene-ethylene/propylene copolymer, a polymethyl pentene polymer, a hydrogenated styrene-ethylene/butylene copolymer, a maleic anhydride functionalized styrene-ethylene/butylene copolymer, a carboxylic acid functionalized styrene-ethylene/butylene copolymer, an acrylonitrile polymer, an acrylonitrile butadiene styrene copolymer, a polypropylene polymer, a polypropylene copolymer, an epoxy resin, a novolac resin, a phenolic resin, a vinyl ester resin, a silicone resin, a nitrile rubber polymer, a natural rubber polymer, a cellulose acetate butyrate polymer, a polyvinyl butyral polymer, an acrylic polymer, an acrylic copolymer or an acrylic copolymer incorporating non-acrylic monomers.

The rigidity, impact and ballistic properties of the articles formed from the fibrous composites of the invention are affected by the tensile modulus of the binder polymers coating the fibers. For example, U.S. Pat. No. 4,623,574 discloses that fiber reinforced composites constructed with elastomeric matrices having tensile moduli less than about 6000 psi (41,300 kPa) have superior ballistic properties compared both to composites constructed with higher modulus polymers, and also compared to the same fiber structure without one or more coatings of a polymeric binder material. However, low tensile modulus polymeric binder polymers also yield lower rigidity composites. Further, in certain applications, particularly those where a composite must function in both anti-ballistic and structural modes, there is needed a superior combination of ballistic resistance and rigidity. Accordingly, the most appropriate type of non-fluorine-containing polymeric binder material to be used will vary depending on the type of article to be formed from the fabrics of the invention. In order to achieve a compromise in both properties, a suitable non-fluorine containing material may combine both low modulus and high modulus materials to form a single polymeric binder material for use as the first polymer layer, as the second polymer layer or as any additional polymer layer. Each polymer layer may also include fillers such as carbon black or silica, may be extended with oils, or may be vulcanized by sulfur, peroxide, metal oxide or radiation cure systems if appropriate, as is well known in the art.

The application of the multilayer coating is conducted prior to consolidating multiple fiber plies, and the multilayer coating is to be applied on top of any pre-existing fiber finish, such as a spin finish. The fibers of the invention may be coated on, impregnated with, embedded in, or otherwise applied with each polymer layer by applying each layer to the fibers, followed by consolidating the coated fiber layers to form a composite. The individual fibers are coated either sequentially or concurrently. Each polymer layer is preferably first applied onto a plurality of fibers followed by forming either a woven fabric or at least one non-woven fiber ply from said fibers. In a preferred embodiment, a plurality of individual fibers are provided as a fiber web, wherein a first polymer layer is applied onto the fiber web, and thereafter a second polymer layer is applied onto the first polymer layer on the fiber web. Thereafter, the coated fiber web is preferably formed into a fabric.

Alternately, a plurality of fibers may first be arranged into a fabric and subsequently coated, or at least one non-woven

## 11

fiber ply may be formed first followed by applying each polymer layer onto each fiber ply. In another embodiment, the fibrous substrate is a woven fabric wherein uncoated fibers are first woven into a woven fabric, which fabric is subsequently coated with each polymer layer. It should be understood that the invention also encompasses other methods of producing fibrous substrates having the multilayer coatings described herein. For example, a plurality of fibers may first be coated with a first polymer layer, followed by forming a woven or non-woven fabric from said fibers, and subsequently applying a second polymer layer onto the first polymer layer on the woven or non-woven fabric. In the most preferred embodiment of the invention, the fibers of the invention are first coated with each polymeric binder material, followed by arranging a plurality of fibers into either a woven or non-woven fabric. Such techniques are well known in the art.

For the purposes of the present invention, the term "coated" is not intended to limit the method by which the polymer layers are applied onto the fibrous substrate surface. Any appropriate method of applying the polymer layers onto substrates may be utilized where the first polymer layer is applied first, followed by subsequently applying the second polymer layer onto the first polymer layer. For example, the polymer layers may be applied in solution form by spraying or roll coating a solution of the polymeric material onto fiber surfaces, wherein a portion of the solution comprises the desired polymer or polymers and a portion of the solution comprises a solvent capable of dissolving the polymer or polymers, followed by drying. Another method is to apply a neat polymer of each coating material to fibers either as a liquid, a sticky solid or particles in suspension or as a fluidized bed. Alternatively, each coating may be applied as a solution, emulsion or dispersion in a suitable solvent which does not adversely affect the properties of fibers at the temperature of application. For example, the fibrous substrate can be transported through a solution of the polymeric binder material to substantially coat the substrate with a first polymeric material and then dried to form a coated fibrous substrate, followed by similarly coating with a second polymeric material. The resulting multilayer coated fiber is then arranged into the desired configuration. In another coating technique, fiber plies or woven fabrics may first be arranged, followed by dipping the plies or fabrics into a bath of a solution containing the first polymeric binder material dissolved in a suitable solvent, such that each individual fiber is at least partially coated with the polymeric binder material, and then dried through evaporation or volatilization of the solvent, and subsequently the second polymer layer may be applied via the same method. The dipping procedure may be repeated several times as required to place a desired amount of polymeric material onto the fibers, preferably encapsulating each of the individual fibers or covering all or substantially all of the fiber surface area with the polymeric material.

Other techniques for applying the coating to the fibers may be used, including coating of the high modulus precursor (gel fiber) before the fibers are subjected to a high temperature stretching operation, either before or after removal of the solvent from the fiber (if using a gel-spinning fiber forming technique). The fiber may then be stretched at elevated temperatures to produce the coated fibers. The gel fiber may be passed through a solution of the appropriate coating polymer under conditions to attain the desired coating. Crystallization of the high molecular weight polymer in the gel fiber may or may not have taken place before the fiber passes into the solution. Alternatively, the fibers

## 12

may be extruded into a fluidized bed of an appropriate polymeric powder. Furthermore, if a stretching operation or other manipulative process, e.g. solvent exchanging, drying or the like is conducted, the coating may be applied to a precursor material of the final fibers. Additionally, the first polymer layer and the second polymer layer may be applied using two different methods.

Preferably, the first and second polymer layers are each applied to the fibrous substrate surfaces when the polymers 10 forming said layers are wet, i.e. in the liquid state. Most preferably, the first polymer and the second polymer are contacted with each other as liquids. In other words, the second polymer is preferably applied onto the fibrous substrate as a liquid while the first polymer is wet. Wet 15 application is preferred. The wet application of each polymer facilitates interlayer adhesion of the polymer layers, wherein the individual layers are unified at the surfaces where they contact each other as polymer molecules from the polymer layers commingle with each other at their 20 contact surfaces and at least partially fuse together. For the purposes of the invention, a liquid polymer includes polymers that are combined with a solvent or other liquid capable of dissolving or dispersing a polymer, as well as molten polymers that are not combined with a solvent or other liquid.

While any liquid capable of dissolving or dispersing a polymer may be used, preferred groups of solvents include water, paraffin oils and aromatic solvents or hydrocarbon solvents, with illustrative specific solvents including paraffin 30 oil, xylene, toluene, octane, cyclohexane, methyl ethyl ketone (MEK) and acetone. The techniques used to dissolve or disperse the coating polymers in the solvents will be those conventionally used for the coating of similar materials on a variety of substrates.

In a most preferred method that has been found to be effective, the first polymer layer and the second polymer layer are first applied onto separate substrates, followed by bringing the substrates together to contact the polymer layers with each other. Most preferably, this method comprises: applying the first polymer onto a surface of a fibrous 35 substrate; applying the second polymer onto a surface of a support; thereafter, joining the fibrous substrate and the support to contact the first polymer with the second polymer; and then separating the support from the fibrous substrate, 40 such that at least a portion of the second polymer is transferred from the support onto the first polymer. The support may be any solid substrate that is capable of supporting a polymer layer, such as a silicone-coated release liner, a solid film or another fabric. The support may also 45 comprise a conveyor belt that is an integral part of utilized fabric processing equipment. The support must be capable of transferring at least a portion of the second polymer onto the first polymer. A preferred method for conducting this technique is described in the examples below and illustrated in 50 FIG. 1.

Generally, a polymeric binder coating is necessary to efficiently merge, i.e. consolidate, a plurality of fiber plies. The multilayer matrix coating may be applied onto the entire surface area of the fibers, or only onto a partial surface area 55 of the fibers. Most preferably, the multilayer matrix coating is applied onto substantially all the surface area of each component fiber of a woven or non-woven fabric of the invention. Where the fabrics comprise a plurality of yarns, each fiber forming a single strand of yarn is preferably coated with the multilayer polymeric binder coating.

When the fibrous substrate is an individual fiber, a plurality of individual fibers may be coated with the multilayer

coating either sequentially or concurrently, and thereafter may be organized into one or more non-woven fiber plies, a non-woven fabric, or woven into a fabric. With regard to woven fabrics, while the matrix coatings may be applied either before or after the fibers are woven, it is most preferred that the matrix coatings be applied after fibers are woven into a fabric due to potential processing limitations. With regard to non-woven fabrics, it is preferred that the polymer coatings be applied before the fibers are formed into a non-woven fabric.

The fibers may be formed into non-woven fabrics which comprise a plurality of overlapping, non-woven fibrous plies that are consolidated into a single-layer, monolithic element. In this embodiment, each ply comprises an arrangement of non-overlapping fibers that are aligned in a unidirectional, substantially parallel array. This type of fiber arrangement is known in the art as a "unitape" (unidirectional tape) and is referred to herein as a "single ply". As used herein, an "array" describes an orderly arrangement of fibers or yarns, and a "parallel array" describes an orderly parallel arrangement of fibers or yarns. A fiber "layer" describes a planar arrangement of woven or non-woven fibers or yarns including one or more plies. As used herein, a "single-layer" structure refers to monolithic structure composed of one or more individual fiber plies that have been consolidated into a single unitary structure. By "consolidating" it is meant that the multilayer polymeric binder coating together with each fiber ply are combined into a single unitary layer. Consolidation can occur via drying, cooling, heating, pressure or a combination thereof. Heat and/or pressure may not be necessary, as the fibers or fabric layers may just be glued together, as is the case in a wet lamination process. The term "composite" refers to combinations of fibers with the multilayer polymeric binder material. Such is conventionally known in the art.

A preferred non-woven fabric of the invention includes a plurality of stacked, overlapping fiber plies (plurality of unitapes) wherein the parallel fibers of each single ply (unitape) are positioned orthogonally (0°/90°) to the parallel fibers of each adjacent single ply relative to the longitudinal fiber direction of each single ply. The stack of overlapping non-woven fiber plies is consolidated under heat and pressure, or by adhering the polymeric resin coatings of individual fiber plies, to form a single-layer, monolithic element which has also been referred to in the art as a single-layer, consolidated network where a "consolidated network" describes a consolidated (merged) combination of fiber plies with a polymeric binder material. The terms "polymeric binder" and "polymeric matrix" are used interchangeably herein, and describe a material that binds fibers together. These terms are conventionally known in the art, and refer to a multilayer material herein.

As is conventionally known in the art, excellent ballistic resistance is achieved when individual fiber plies are cross-plied such that the fiber alignment direction of one ply is rotated at an angle with respect to the fiber alignment direction of another ply. Most preferably, the fiber plies are cross-plied orthogonally at 0° and 90° angles, but adjacent plies can be aligned at virtually any angle between about 0° and about 90° with respect to the longitudinal fiber direction of another ply. For example, a five ply non-woven structure may have plies oriented at a 0°/45°/90°/45°/0° or at other angles. Such rotated unidirectional alignments are described, for example, in U.S. Pat. Nos. 4,457,985; 4,748,064; 4,916,000; 4,403,012; 4,623,573; and 4,737,402.

Most typically, non-woven fabrics include from 1 to about 6 plies, but may include as many as about 10 to about 20

plies as may be desired for various applications. The greater the number of plies translates into greater ballistic resistance, but also greater weight. Accordingly, the number of fiber plies forming a fabric or an article of the invention varies depending upon the ultimate use of the fabric or article. For example, in body armor vests for military applications, in order to form an article composite that achieves a desired 1.0 pound per square foot areal density (4.9 kg/m<sup>2</sup>), a total of at 22 individual plies may be required, 10 wherein the plies may be woven, knitted, felted or non-woven fabrics (with parallel oriented fibers or other arrangements) formed from the high-strength fibers described herein. In another embodiment, body armor vests for law enforcement use may have a number of plies based on the 15 National Institute of Justice (NIJ) Threat Level. For example, for an NIJ Threat Level IIIA vest, there may also be a total of 22 plies. For a lower NIJ Threat Level, fewer plies may be employed.

Further, the fiber plies of the invention may alternately 20 comprise yarns rather than fibers, where a "yarn" is a strand consisting of multiple fibers or filaments. Non-woven fiber plies may alternately comprise other fiber arrangements, such as felted structures which are formed using conventionally known techniques, comprising fibers in random 25 orientation instead of parallel arrays. Articles of the invention may also comprise combinations of woven fabrics, non-woven fabrics formed from unidirectional fiber plies and non-woven felt fabrics.

Consolidated non-woven fabrics may be constructed 30 using well known methods, such as by the methods described in U.S. Pat. No. 6,642,159, the disclosure of which is incorporated herein by reference. As is well known in the art, consolidation is done by positioning the individual fiber plies on one another under conditions of sufficient heat and 35 pressure to cause the plies to combine into a unitary fabric. Consolidation may be done at temperatures ranging from about 50° C. to about 175° C., preferably from about 105° C. to about 175° C., and at pressures ranging from about 5 psig (0.034 MPa) to about 2500 psig (17 MPa), for from 40 about 0.01 seconds to about 24 hours, preferably from about 0.02 seconds to about 2 hours. When heating, it is possible 45 that the polymeric binder coatings can be caused to stick or flow without completely melting. However, generally, if the polymeric binder materials are caused to melt, relatively little pressure is required to form the composite, while if the binder materials are only heated to a sticking point, more pressure is typically required. As is conventionally known in the art, consolidation may be conducted in a calender set, a flat-bed laminator, a press or in an autoclave.

Alternately, consolidation may be achieved by molding 50 under heat and pressure in a suitable molding apparatus. Generally, molding is conducted at a pressure of from about 50 psi (344.7 kPa) to about 5000 psi (34470 kPa), more preferably about 100 psi (689.5 kPa) to about 1500 psi 55 (10340 kPa), most preferably from about 150 psi (1034 kPa) to about 1000 psi (6895 kPa). Molding may alternately be conducted at higher pressures of from about 500 psi (3447 kPa) to about 5000 psi, more preferably from about 750 psi (5171 kPa) to about 5000 psi and more preferably from 60 about 1000 psi to about 5000 psi. The molding step may take from about 4 seconds to about 45 minutes. Preferred molding temperatures range from about 200° F. (~93° C.) to about 350° F. (~177° C.), more preferably at a temperature from about 200° F. to about 300° F. (~149° C.) and most preferably 65 at a temperature from about 200° F. to about 280° F. (~121° C.). The pressure under which the fabrics of the invention are molded has a direct effect on the stiffness or

flexibility of the resulting molded product. Particularly, the higher the pressure at which the fabrics are molded, the higher the stiffness, and vice-versa. In addition to the molding pressure, the quantity, thickness and composition of the fabric plies and polymeric binder coating types also directly affects the stiffness of the articles formed from the inventive fabrics.

While each of the molding and consolidation techniques described herein are similar, each process is different. Particularly, molding is a batch process and consolidation is a continuous process. Further, molding typically involves the use of a mold, such as a shaped mold or a match-die mold when forming a flat panel, and does not necessarily result in a planar product. Normally consolidation is done in a flat-bed laminator, a calendar nip set or as a wet lamination to produce soft body armor fabrics. Molding is typically reserved for the manufacture of hard armor, e.g. rigid plates. In the context of the present invention, consolidation techniques and the formation of soft body armor are preferred.

In either process, suitable temperatures, pressures and times are generally dependent on the type of polymeric binder coating materials, polymeric binder content (of the combined coatings), process used and fiber type. The fabrics of the invention may optionally be calendered under heat and pressure to smooth or polish their surfaces. Calendering methods are well known in the art.

Woven fabrics may be formed using techniques that are well known in the art using any fabric weave, such as plain weave, crowfoot weave, basket weave, satin weave, twill weave and the like. Plain weave is most common, where fibers are woven together in an orthogonal 0°/90° orientation. In another embodiment, a hybrid structure may be assembled where both woven and non-woven fabrics are combined and interconnected, such as by consolidation. Prior to weaving, the individual fibers of each woven fabric material may or may not be coated with the first polymer layer and second polymer layer, or other additional polymer layers.

To produce a fabric article having sufficient ballistic resistance properties, the proportion of fibers forming the fabric preferably comprises from about 50% to about 98% by weight of the fibers plus the weight of the combined polymeric coatings, more preferably from about 70% to about 95%, and most preferably from about 78% to about 90% by weight of the fibers plus the polymeric coatings. Thus, the total weight of the combined polymeric coatings preferably comprises from about 2% to about 50% by weight of the fabric, more preferably from about 5% to about 30% and most preferably from about 10% to about 22% by weight of the fabric, wherein 16% is most preferred.

The thickness of the individual fabrics will correspond to the thickness of the individual fibers. A preferred woven fabric will have a preferred thickness of from about 25 µm to about 500 µm per layer, more preferably from about 50 µm to about 385 µm and most preferably from about 75 µm to about 255 µm per layer. A preferred non-woven fabric, i.e. a non-woven, single-layer, consolidated network, will have a preferred thickness of from about 12 µm to about 500 µm, more preferably from about 50 µm to about 385 µm and most preferably from about 75 µm to about 255 µm, wherein a single-layer, consolidated network typically includes two consolidated plies (i.e. two unitapes). While such thicknesses are preferred, it is to be understood that other thicknesses may be produced to satisfy a particular need and yet fall within the scope of the present invention.

The fabrics of the invention will have a preferred areal density of from about 50 grams/m<sup>2</sup> (gsm) (0.01 lb/ft<sup>2</sup> (psf)

to about 1000 gsm (0.2 psf). More preferable areal densities for the fabrics of this invention will range from about 70 gsm (0.014 psf) to about 500 gsm (0.1 psf). The most preferred areal density for fabrics of this invention will range from about 100 gsm (0.02 psf) to about 250 gsm (0.05 psf). The articles of the invention, which comprise multiple individual layers of fabric stacked one upon the other, will further have a preferred areal density of from about 1000 gsm (0.2 psf) to about 40,000 gsm (8.0 psf), more preferably from about 10 2000 gsm (0.40 psf) to about 30,000 gsm (6.0 psf), more preferably from about 3000 gsm (0.60 psf) to about 20,000 gsm (4.0 psf), and most preferably from about 3750 gsm (0.75 psf) to about 10,000 gsm (2.0 psf).

The composites of the invention may be used in various 15 applications to form a variety of different ballistic resistant articles using well known techniques. For example, suitable techniques for forming ballistic resistant articles are described in, for example, U.S. Pat. Nos. 4,623,574, 4,650, 710, 4,748,064, 5,552,208, 5,587,230, 6,642,159, 6,841,492 20 and 6,846,758. The composites are particularly useful for the formation of flexible, soft armor articles, including garments such as vests, pants, hats, or other articles of clothing, and covers or blankets, used by military personnel to defeat a number of ballistic threats, such as 9 mm full metal jacket 25 (FMJ) bullets and a variety of fragments generated due to explosion of hand-grenades, artillery shells, Improvised Explosive Devices (IED) and other such devices encountered in a military and peace keeping missions. As used herein, "soft" or "flexible" armor is armor that does not 30 retain its shape when subjected to a significant amount of stress and is incapable of being free-standing without collapsing. The composites are also useful for the formation of rigid, hard armor articles. By "hard" armor is meant an article, such as helmets, panels for military vehicles, or 35 protective shields, which have sufficient mechanical strength so that it maintains structural rigidity when subjected to a significant amount of stress and is capable of being free-standing without collapsing. Fabric composites can be cut into a plurality of discrete sheets and stacked for formation 40 into an article or they can be formed into a precursor which is subsequently used to form an article. Such techniques are well known in the art.

Garments may be formed from the composites of the 45 invention through methods conventionally known in the art. Preferably, a garment may be formed by adjoining the ballistic resistant fabric composites of the invention with an article of clothing. For example, a vest may comprise a generic fabric vest that is adjoined with the ballistic resistant composites of the invention, whereby the inventive composites are inserted into strategically placed pockets. This 50 allows for the maximization of ballistic protection, while minimizing the weight of the vest. As used herein, the terms "adjoining" or "joined" are intended to include attaching, such as by sewing or adhering and the like, as well as un-attached coupling or juxtaposition with another fabric, such that the ballistic resistant materials may optionally be 55 easily removable from the vest or other article of clothing. Articles used in forming flexible structures like flexible sheets, vests and other garments are preferably formed from using a low tensile modulus binder material. Hard articles like helmets and armor are preferably formed using a high tensile modulus binder material.

Ballistic resistance properties are determined using standard testing procedures that are well known in the art. 60 Particularly, the protective power or penetration resistance of a ballistic resistant composite is normally expressed by citing the impacting velocity at which 50% of the projectiles

17

penetrate the composite while 50% are stopped by the shield, also known as the  $V_{50}$  value. As used herein, the "penetration resistance" of an article is the resistance to penetration by a designated threat, such as physical objects including bullets, fragments, shrapnel and the like, and non-physical objects, such as a blast from explosion. For composites of equal areal density, which is the weight of the composite divided by its area, the higher the  $V_{50}$ , the better the ballistic resistance of the composite. The ballistic resistant properties of the articles of the invention will vary depending on many factors, particularly the type of fibers used to manufacture the fabrics, the percent by weight of the fibers in the composite, the suitability of the physical properties of the matrix materials, the number of layers of fabric making up the composite and the total areal density of the composite. However, the use of one or more polymeric coatings that are resistant to dissolution or penetration by sea water, and resistant to dissolution or penetration by one or more organic solvents, does not negatively affect the ballistic properties of the articles of the invention.

The following examples serve to illustrate the invention:

## EXAMPLE 1

A silicone-coated release paper support is coated with a polymeric binder material that is a water-based acrylic dispersion of HYCAR® T122 (commercially available from Noveon, Inc. of Cleveland, Ohio) using a standard pan-fed reverse roll coating method. The polymeric binder material was applied at full strength.

Separately, a fibrous web comprising aramid yarns (TWARON® 1000-denier, type 2000 aramid yarns, commercially available from Teijin Twaron BV of The Netherlands) is coated with the same water-based acrylic dispersion of HYCAR® T122 in a yarn impregnator using a dip and squeeze technique.

A schematic illustration of this hybrid coating technique is provided in FIG. 1. In the pan-fed reverse roll coating method, a metering roller and an application roller are positioned in parallel at a pre-determined fixed distance from each other. Each roller has approximately the same physical dimensions. The rollers are held at the same elevation and their bottoms are submerged in a liquid resin bath of the polymeric binder material contained in a pan. The metering roller is held stationary while the applicator roller is rotated in a direction that would lift some of the liquid in the resin bath towards the gap between the rollers. Only the amount of liquid that will fit through this gap is carried to the upper surface of the applicator roll, and any excess falls back into the resin bath.

Concurrently, the support is carried towards the upper surface of the applicator roll, with its direction of travel being opposite to the direction the upper surface of the rotating applicator roll. When the support is directly above the applicator roll, it is pressed onto the upper surface of the applicator roller by means of a backing roller. All of the liquid that is carried by the upper surface of the applicator roller is then transferred to the support. This technique is used to apply a precisely metered amount of liquid resin to the surface of the silicone-coated release paper.

The dip and squeeze technique is conducted to coat the fibrous web with the diluted resin dispersion using the following steps:

1. Spools of TWARON® yarn are unwound from a creel.
2. The yarns are sent through a though a series of combs, which cause the yarns to be evenly spaced and parallel

18

to each other. At this point, the individual yarns are closely positioned and parallel to one another in a substantially parallel array.

3. The substantially parallel array is then passed over a series of rotating idler rollers that redirect the substantially parallel array down and through the liquid resin bath. In this bath, each of the yarns is completely submerged into the liquid for a length of time sufficient to cause the liquid to penetrate each yarn bundle, wetting the individual fibers or filaments within the yarn.
  4. At the end of this liquid resin bath, the wetted fibrous web is pulled over a series of stationary (non-rotating) spreader bars. The spreader bars spread out the individual yarns until they abut or overlap with their neighbors. Before spreading, the cross-sectional shape of each yarn bundle is approximately round. After spreading, the cross-sectional shape of each yarn bundle is approximately elliptical, tending towards a rectangle shape. An ultimate spread would be for each fiber or filament to be next to one another in a single fiber plane.
  5. Once the wetted fibrous web passes over the last spreader bar, it is again re-directed, this time up and out of the liquid. This wetted fibrous web then is wrapped around a large rotating idler roller. The fibrous web carries with it an excess of the liquid.
  6. In order to remove this excess liquid from the fibrous web, another freely rotating idler roller is positioned to ride on the surface of the large rotating idler roller. These two idler rollers are parallel to each other and the freely rotating idler roller is mounted in such a way that it bears down on the large rotating idler roller in a radial direction, effectively forming a nip. The wetted fibrous web is carried through this nip and the force applied by the freely rotating idler roller acts to squeeze off the excess liquid, which runs back into the liquid resin bath.
- At this point, the coated fibrous web and the coated silicone-coated release paper are brought into contact with one another on the "combining roller". The wetted (impregnated) fibrous web is cast onto the wet side of the silicone-coated release paper and passed over the combining roller such that the NUVA® LB-coated aramid fiber web is pressed into the wet coating of HYCAR® T122 that is carried on the surface of the silicone-coated release paper. The assembly is then passed through an oven to dry off the water.
- A series of squares are cut from this unidirectional tape ("UDT"). Two squares are then oriented fiber-side to fiber-side and one of the squares is rotated so that the direction of its fibers is perpendicular to the fiber direction of the first square. These pairs of configured squares are then placed into a press, and subjected to 240° F. (115.56° C.) and 100 PSI (689.5 kPa) for 15 minutes. The press is then cooled to room temperature and the pressure is released. The squares are now bonded to one another. The release paper is removed from both sides of this composite, resulting in a single layer of a non-woven fabric. This procedure is repeated to produce additional layers as needed for ballistic testing.

## EXAMPLE 2

Example 1 is repeated by replacing the water-based acrylic dispersion of HYCAR® T122 with a dilute water-based dispersion of a fluorine-containing resin (NUVA®

## 19

LB, commercially available from Clariant International, Ltd. of Switzerland; dilution: 10% of Nuva LB, 90% de-ionized water).

While the present invention has been particularly shown and described with reference to preferred embodiments, it will be readily appreciated by those of ordinary skill in the art that various changes and modifications may be made without departing from the spirit and scope of the invention. It is intended that the claims be interpreted to cover the disclosed embodiment, those alternatives which have been discussed above and all equivalents thereto.

What is claimed is:

1. A ballistic resistant fibrous composite comprising at least one fibrous substrate having a multilayer coating thereon, wherein said fibrous substrate comprises one or more yarn bundles having a tenacity of about 7 g/denier or more and a tensile modulus of about 150 g/denier or more, each yarn bundle comprising a plurality of fibers; said multilayer coating comprising a first polymer layer on a surface of said fibers, said first polymer layer comprising a first polymer, and a second polymer layer on said first polymer layer, said second polymer layer comprising a second polymer, wherein the first polymer and the second polymer are the same and comprise a blend of a nitrile rubber and a fluoropolymer, wherein said fluoropolymer comprises a polychlorotrifluoroethylene homopolymer, a chlorotrifluoroethylene copolymer, an ethylene-chlorotrifluoroethylene copolymer, an ethylene-tetrafluoroethylene copolymer, a fluorinated ethylene-propylene copolymer, perfluoroalkoxyethylene, polytetrafluoroethylene, polyvinyl fluoride, polyvinylidene fluoride, a fluorocarbon-modified polyether, a fluorocarbon-modified polyester, a fluorocarbon-modified polyanion, a fluorocarbon-modified polyacrylic acid, a fluorocarbon-modified polyacrylate, a fluorocarbon-modified polyurethane, or a copolymer or a blend thereof, wherein at least the first polymer layer penetrates each yarn bundle and coats the individual fibers within each yarn bundle, and wherein the multilayer coating comprises at least one additional polymer layer on the second polymer layer, wherein the at least one additional polymer layer is different than the first polymer layer and the second polymer layer,

and wherein the total weight of the combined polymeric coatings comprises from about 10% to about 22% by weight of the composite.

2. A ballistic resistant fibrous composite comprising at least one fibrous substrate having a multilayer coating thereon, wherein said fibrous substrate comprises one or more yarn bundles having a tenacity of about 7 g/denier or more and a tensile modulus of about 150 g/denier or more, each yarn bundle comprising a plurality of fibers; wherein said multilayer coating consists of a first polymer layer on a surface of said fibers, said first polymer layer consisting of a first polymer, wherein the first polymer consists of a single polymer or a single co-polymer, and a second polymer layer on said first polymer layer, said second polymer layer consisting of a second polymer, wherein the second polymer consists of a single polymer or a single co-polymer, wherein the first polymer and the second polymer are the same and wherein each of the first polymer and second polymer consist of a polychlorotrifluoroethylene homopolymer, a chlorotrifluoroethylene copolymer, an ethylene-chlorotrifluoroethylene copolymer, an ethylene-tetrafluoroethylene

## 20

copolymer, a fluorinated ethylene-propylene copolymer, perfluoroalkoxyethylene, polytetrafluoroethylene, polyvinyl fluoride, polyvinylidene fluoride, fluorocarbon-modified polyethers, fluorocarbon-modified polyesters, fluorocarbon-modified polyanions, fluorocarbon-modified polyacrylic acid, fluorocarbon-modified polyacrylates, fluorocarbon-modified polyurethanes, or a copolymer thereof, wherein at least the first polymer layer penetrates each yarn bundle and coats the individual fibers within each yarn bundle.

3. The ballistic resistant fibrous composite of claim 2 wherein the composite consists of at least one fibrous substrate having said multilayer coating thereon, wherein said fibrous substrate consists of one or more yarn bundles having a tenacity of about 7 g/denier or more and a tensile modulus of about 150 g/denier or more, each yarn bundle consisting of a plurality of fibers.

4. A ballistic resistant fibrous composite comprising at least one fibrous substrate having a multilayer coating thereon, wherein said fibrous substrate comprises one or more yarn bundles having a tenacity of about 7 g/denier or more and a tensile modulus of about 150 g/denier or more, each yarn bundle comprising a plurality of fibers; said multilayer coating comprising a first polymer layer on a surface of said fibers, said first polymer layer comprising a first polymer, and a second polymer layer on said first polymer layer, said second polymer layer comprising a second polymer, wherein the first polymer and the second polymer are the same and comprise a blend of a nitrile rubber and a fluoropolymer.

5. The ballistic resistant fibrous composite of claim 4 wherein said fluoropolymer comprises a polychlorotrifluoroethylene homopolymer, a chlorotrifluoroethylene copolymer, an ethylene-chlorotrifluoroethylene copolymer, an ethylene-tetrafluoroethylene copolymer, a fluorinated ethylene-propylene copolymer, perfluoroalkoxyethylene, polytetrafluoroethylene, polyvinyl fluoride, polyvinylidene fluoride, a fluorocarbon-modified polyether, a fluorocarbon-modified polyester, a fluorocarbon-modified polyanion, a fluorocarbon-modified polyacrylic acid, a fluorocarbon-modified polyacrylate, a fluorocarbon-modified polyurethane, or a copolymer or a blend thereof.

6. The ballistic resistant fibrous composite of claim 5 wherein at least the first polymer layer penetrates each yarn bundle and coats the individual fibers within each yarn bundle.

7. The ballistic resistant fibrous composite of claim 4 wherein at least the first polymer layer penetrates each yarn bundle and coats the individual fibers within each yarn bundle.

8. The ballistic resistant fibrous composite of claim 4 wherein the multilayer coating comprises at least one additional polymer layer on the second polymer layer, wherein the at least one additional polymer layer is different than the first polymer layer and the second polymer layer.

9. The ballistic resistant fibrous composite of claim 4 wherein the total weight of the combined polymeric coatings comprises from about 10% to about 22% by weight of the composite.

10. The ballistic resistant fibrous composite of claim 3 and wherein the total weight of the combined polymeric coatings comprises from about 10% to about 22% by weight of the composite.